

Patented Jan. 8, 1929.

1,698,705

# UNITED STATES PATENT OFFICE.

SHINJIRO HORII, OF TOKYO, JAPAN.

## STENCIL SHEET.

No Drawing.

Application filed May 18, 1926. Serial No. 109,973.

This invention relates to improvements in stencil sheets of the type commonly used for autographic and typewriting duplication, consisting of a sheet of fibrous material coated or impregnated with a coating material including phenolic resins and esters of polysaccharides.

The object of the present invention is to provide an improved stencil sheet which offers a considerably great resistance to the atmospheric influences on using or storing, and gives a large number of clear and sharp copies.

In carrying out the invention a base of open-texture, porous material of any suitable character, such as yoshino paper is coated or impregnated with a coating material prepared by mixing together a solution of a phenolic resin in a suitable solvent, such as alcohol, with a solution of esters of polysaccharides, such as cellulose nitrate, cellulose acetate and mannan acetate, in a suitable solvent, such as acetone, alcohol and amyl acetate.

The phenolic resin is a condensation product of phenols and formaline or other aldehydes in the presence of a small amount of alkalies or acids on application of heat, and which is soluble in alcohol.

In the present invention other artificial or natural resins, such as coumarone resin, ester gum, colophony and shellac, may be added to the coating material. And, if necessary, a suitable proportion of a tempering agent, such as oils, fats, fatty acids and waxes, and coloring matters, such as a dye or a pigment, may be added to the above described coating material.

The yoshino paper may be coated or impregnated with the solution above described in any desired manner; or the composition may be added into the paper stuff in a mixing hollander.

The proportions of the ingredients of the composition may vary according to several circumstances, an example being as follows:—

|                                | Parts<br>by weight. |
|--------------------------------|---------------------|
| Phenolic resin, 20% solution   | 200                 |
| Cellulose nitrate, 5% solution | 100                 |
| Stearine                       | 10                  |
| Castor oil                     | 20                  |

The term "esters of polysaccharides" is in-

tended to include not only one of definite esters of polysaccharides, but also a mixture of them.

The wax-coated stencil sheet which hitherto commonly used, has the great disadvantages of being liable to pass the ink through the cracks caused accidentally by the usual handling, and particularly sensitive to the action of heat. Other kinds of improved flexible stencil sheets are obtained by employing certain protein substances, particularly gelatine. It is very troublesome to preliminarily moisten the sheet in order to adapt it for making the stencil by pressure. Moreover the iron parts of the writing machine are very injuriously affected by the moisture of the sheets.

According to the present invention the porous base is coated or impregnated with a material, not hitherto employed for this purpose, including phenolic resin and esters of polysaccharides. The coated sheet, as above described, being soft and flexible remains throughout an extended period of time practically unchanged without the drawback of becoming sticky or friable. By the pressure of a hand stylus or the blow of the type of a writing machine without moistening the sheet the clear characters may be easily produced thereon.

What I claim is:—

1. In a stencil sheet, the combination with a base of fibrous material, of an impregnating composition comprising resin, esters of polysaccharides and a tempering agent.

2. In a stencil sheet, the combination with a base of fibrous material, of an impregnating composition comprising a phenolic resin, esters of polysaccharides and a tempering agent.

3. A stencil sheet composed of a base of fibrous material and an impregnating composition comprising a phenolic resin, cellulose nitrate, stearine and castor oil.

4. A stencil sheet as specified in claim 3, in which the said composition comprises the said substances in the following proportion:

|                                |     |
|--------------------------------|-----|
| Phenolic resin, 20% solution   | 200 |
| Cellulose nitrate, 5% solution | 100 |
| Stearine                       | 10  |
| Castor oil                     | 20  |

In testimony whereof I affix my signature.  
SHINJIRO HORII.